

## UNITED STATES PATENT OFFICE

2,352,099

## TISSUE FILLER

George E. Hobdell, Upper Darby, Pa.

No Drawing. Application May 12, 1942.  
Serial No. 442,578

4 Claims. (Cl. 27—21)

My invention relates to a new and useful slowly solidifying chemical solution for use as a tissue filler in connection with the treatment of corpses.

The human body after death, in many cases, is emaciated, due to prolonged illness but depending largely upon the sickness from which death resulted, and from other causes.

To aid the undertakers in restoring as natural appearance as possible to the deceased it is necessary to cause the tissues to be built up in such a manner as not to distort the features any more than possible.

The improvement herein described provides a slowly solidifying solution which, when injected into a body or corpse by the use of any suitable hypodermic needle or syringe, will begin to solidify upon contact with the tissue fluids or the moisture contained therein and form a pliable mass that can be so molded as to restore, as nearly as possible, the likeness in the face and head of the deceased before the fatal illness.

One of the advantages of the present invention is that the filler slowly solidifies so that prior to solidification taking place it assumes a plastic state and remains in this condition a sufficient length of time to permit an operator to model the features of the corpse in a manner somewhat similar to a sculptor working clay which will result in a lifelike appearance.

In order that those skilled in the art to which this invention appertains may understand how to make and use the same I will describe the product in detail.

In carrying out the invention as herein embodied I produce a tissue filler for corpses comprising a solution of water insoluble cellulosic material in a highly water soluble solvent, the formula thereof being as follows:

|                              | c. c. |
|------------------------------|-------|
| Nitrocellulose (nitrocotton) | 90    |
| Methanol (over 99% pure)     | 3840  |
| Formaldehyde solution        | 40    |
| Glycerine (U. S. P.)         | 60    |
| Jasamin                      | 6     |
| Chypre                       | 3     |
| Eosine dye                   | 15    |

It is understood that the particulars herein given are in no way limitative, and that while still keeping within the scope of the invention any desired modification or proportions may be

made in the solution according to the circumstances.

The method of building up the tissues of an emaciated corpse includes the injecting of a quantity of the solution into the tissues by the use of a hypodermic needle or syringe causing the solution to contact the tissue fluids, or the moisture therein, and thereby be dispersed in the tissues to precipitate a readily moldable tissue filler that is manually kneaded into suitable and proper formations.

This particular method of building or filling up the tissues of an emaciated corpse comprises the injecting of a nitrocellulose in methanol solution including formaldehyde solution and glycerine in particular, and in combination with the other ingredients constitutes a readily moldable tissue builder. The glycerine contained in the product especially limits dehydration or deterioration of the moldable mass thus formed, provides a more pliable and workable substance for the embalmer or other operator while the addition of the formaldehyde solution preserves the tissues not affected by the embalming fluids used.

Of course I do not wish to be limited to the exact quantities or proportions of the ingredients set forth as these may be varied within the scope of the appended claims without departing from the spirit of my invention.

Having thus described my invention what I claim as new and useful is:

1. A tissue filler for corpses comprising 90 c. c. nitrocellulose, 3840 c. c. methanol (over 99% pure), 40 c. c. formaldehyde solution, 60 c. c. glycerine, 6 c. c. jasamin, 3 c. c. chypre, and 15 c. c. eosine dye.

2. A tissue filler for corpses comprising approximately 90 c. c. nitrocellulose, 3840 c. c. methanol, 40 c. c. formaldehyde solution, and 60 c. c. glycerine.

3. A tissue filler for corpses comprising a solution of nitrocellulose in methanol of approximately forty-three parts of methanol to one of nitrocellulose, glycerine, and formaldehyde solution.

4. A tissue filler for corpses comprising 90 c. c. nitrocellulose, 3840 c. c. methanol, 40 c. c. formaldehyde solution, and sufficient glycerine to retard the solidification of the nitrocellulose.

GEO. E. HOBDELL.